

April 7, 1931.

H. GERDIEN ET AL

1,799,225

SPARK PLUG

Filed Dec. 8, 1928

FIG. 1



FIG. 2



Inventors

Hans Gerdien, &  
Reinhold Reichmann

by *Knight Bry* *attorneys*

## UNITED STATES PATENT OFFICE

HANS GERDIEN, OF BERLIN-GRUNEWALD, AND REINHOLD REICHMANN, OF BERLIN, GERMANY, ASSIGNEES TO SIEMENS & HALSKE, AKTIENGESELLSCHAFT, OF SIEMENSSTADT, NEAR BERLIN, A CORPORATION OF GERMANY

## SPARK PLUG

Application filed December 8, 1928, Serial No. 324,604, and in Germany December 23, 1927.

Our invention relates to improvements in spark plugs.

It is already known to construct the insulators of spark plugs of quartz, if preferred in two parts. It has, for instance, been proposed to construct the lower part only of the insulator, adjacent to the spark gap and subjected to the highest temperatures, of quartz.

According to our invention at least that part of a two-part insulator of a spark plug which is adjacent to the spark gap, or the end facing the combustion chamber of the engine, is constructed of aluminum-oxide. The insulator may be constructed of aluminum-oxide produced from sintered or fused aluminum-oxide, such as artificial sapphire or ruby. Sintered and fused aluminum-oxide is indifferent to temperature fluctuations, like quartz glass. It is, further, at the high temperatures in question less subject to reactions, so that its surface facing the combustion chamber is not attacked in any way. It may be advisable to polish this surface, so that any particles of carbon precipitated upon it are easily dislodged and thus the plug does not become choked by carbon deposits.

In the drawings attached hereto and forming part of our specification two embodiments of our invention are illustrated by way of example.

In the drawings—

Fig. 1, represents a longitudinal section through one construction of our improved spark plug, and

Fig. 2, a longitudinal section through a modification of the plug.

Referring to Fig. 1 of the drawings, 1 is the part of the insulator directly exposed to the hot products of combustion in the engine, which part according to our invention is constructed of aluminum-oxide. 2 is the main portion of the insulator, mounted in the socket 4 by means of the packings 3 in the customary manner. The central electrode 5 is provided with a collar or shoulder 6. The main portion 2 of the insulator and the tip 1 are joined between this collar 6 and a clamping device, such as a nut, located at the outer 50 end of the ignition electrode.

Fig. 2 illustrates at 7 a different design of the insulator portion, which according to our invention is constructed of aluminum-oxide. The remaining parts of the spark plug are assumed to be similar to those shown in Fig. 1 and are indicated by the like numerals of reference. The end of the insulator portion 7 is outwardly and inwardly tapered and is provided at its thicker end with a flange, which abuts against the main portion 2 of the insulator. The surface of the tapering part 7 is preferably highly finished, so that no carbon or the like can adhere to it.

On account of the high costs caused by machining fused aluminum-oxide, the insulator tip is preferably produced by sintering aluminum-oxide at temperatures of more than 1600° C.

The manufacture of sintered insulators for spark plugs is preferably carried out in the following manner:

The aluminum-oxide is, prior to the sintering process, moulded by one of the methods known in the art, dried and then sintered, preferably at temperatures as near as possible to the melting point of aluminum-oxide, such as 1900° C. The period of sintering is so chosen, that the insulator produced has a marble-like appearance imparted to it. As a rule, several hours are necessary to obtain this result. The insulator then hardly differs from those made of fused aluminum-oxide regarding its refractory and insulating qualities. Its production is, however, far less expensive, because the high costs of machining are eliminated.

The manufacture of the insulator may be started from ordinary aluminum-oxide as well as from an oxide which has been subjected to a preliminary fusing. As it is comparatively easy to produce large-size insulators by sintering, not only the portion of the insulator subject to the highest temperatures should be made of aluminum-oxide sintered at over 1600° C., but the entire insulator.

Careful tests have proven that aluminum oxide for insulators produced as described hereinbefore is superior to all other materials:

1. On account of its high resistance to 100

chemical attacks by combustion products in the cylinder, in particular also its resistivity to so-called anti-knocking metal compounds now frequently added to the fuel, because aluminum oxide does not form compounds with these combustion products. It should be noted that for instance the glazing of porcelain insulators which consists of silicates will form compounds with the combustion products, and accordingly in time will be destroyed.

2. On account of the high refractory qualities so that it may be allowed to heat to the point where no carbon deposit could form on it. Also in this respect porcelain cannot fulfill this requirement.

3. On account of its great heat conductivity. Also in this respect the porcelain insulator fails.

4. On account of its small heat expansion, so that it will not crack at quick variations in temperature. Porcelain insulators are well known to crack at quick variations in temperature.

5. On account of its high electric insulating quality not impaired by chemical reactions with the combustion products. Also this requirement is not fulfilled by porcelain.

6. Aluminum oxide has great density rendering it impermeable to gases, and

7. It is easily molded into any desirable form in unsintered condition and, therefore, easily manufactured by sintering at high temperatures. With respect to points 6 and 7 porcelain would fulfill these requirements inasmuch as porcelain has great density, and when glazed is impermeable to gases and can be molded before it is fired.

In some of the annexed claims we have characterized the insulator as "consisting substantially entirely of aluminum oxide", by which we mean that the insulator thus produced consists of substantially pure aluminum oxide, excepting such impurities as would not have any effect upon the aforementioned properties.

The use of our insulator of fused or sintered aluminum-oxide is particularly advantageous, if the internal combustion engine is fed with fuel containing metal compounds, and in which the precipitation of conducting layers upon the insulator is easily possible. The insulator consisting of aluminum-oxide may be provided in well known manner with petticoats in order to increase the length of the creeping path.

Various modifications and changes may be made without departing from the spirit and the scope of the invention.

60 We claim as our invention:

1. A spark plug, comprising conducting electrodes and an insulator consisting substantially entirely of aluminum-oxide.

65 2. A spark plug, comprising conducting electrodes, and an insulator serving for

mounting said electrodes, said insulator consisting at the end facing the combustion chamber substantially entirely of aluminum-oxide.

3. A spark plug, comprising conducting electrodes and an insulator consisting of sintered aluminum-oxide.

4. A spark plug, comprising conducting electrodes and an insulator for mounting said electrodes, said insulator consisting at least at the end facing the combustion chamber of the engine of sintered aluminum-oxide.

5. A spark plug, comprising conducting electrodes and an insulator consisting substantially entirely of aluminum oxide, sintered at suitable temperatures to form a substantially crystalline body.

6. A spark plug, comprising conducting electrodes and an insulator for mounting said electrodes, said insulator consisting at the end facing the combustion chamber substantially entirely of aluminum oxide sintered at suitable temperatures to form a substantially crystalline body.

In testimony whereof we affix our signatures.

HANS GERDIEN.  
REINHOLD REICHMANN.

70

75

80

85

95

100

105

110

115

120

125

130